# EUROPEAN PATENT SPECIFICATION

(11) **EP 0 337 425 B1**
(45) Date of publication and mention of the grant of the patent: **16.10.1991**
(21) Application number: 89106508.8
(22) Date of filing: 12.04.1989
(51) Int. Cl.: C10M 169/04

(54) **Antirust additives for lubricants or greases based on perfluoropolyethers**
Antirostadditive für Schmiermittel oder Schmierfette mit Perfluoropolyäthern als Basismaterial
Additifs antirouilles pour lubrifiants ou graisses à base de perfluoropolyéthers

(30) Priority: 13.04.1988 IT 2018388
(43) Date of publication of application: 18.10.1989
(73) Proprietor: AUSIMONT S.r.l., I-20100 Milano (IT)
(72) Inventor: Strepparola, Ezio, I-24047 Treviglio Bergamo (IT); Gavezotti, Piero, I-20100 Milan (IT); Corti, Costante, I-20100 Milan (IT)
(74) Representative: Barz, Peter, Dr.

(56) References cited:
- DE-A- 2 632 837
- US-A- 4 085 137
- US-A- 4 132 660
- US-A- 4 194 983
- US-A- 4 404 377

## Description

The present invention relates to functionalized fluoropolyether compounds which impart antirust properties to lubricating oils and greases based on perfluoropolyethers.

It is known that the utilization of perfluoropolyethers as lubricants does not prevent the formation of rust on the surface of ferrous materials when moisture is present, even if said materials are covered with an oil film.

This is due to the high permeability to gases, vapours and, among these, also to water vapour, exhibited by perfluoropolyethers (PFPE).

PFPE utilizable also for formulating lubricating oils and greases are well-known on the market, for example, Fomblin^{(R)} (produced by Montedison), KRYTOX^{(R)} (produced by DuPont), DENNUM^{(R)} (produced by Daikin), and the like.

It is known that it is very difficult to add substances to said PFPE because a characteristic thereof is their absolute immiscibility with most of the chemical compounds. Consequently, in the case of PFPE lubricants, it is impossible to use the products usually added as antirust additives for mineral oils (which are the traditional lubricants) which form stable mixtures with each other.

The compounds according to the present invention represent a significant improvement in antirust protection as compared with the anticorrosive products described in EP-A-95825, 165649, 165650 and IT-A-20159 A/86.

In particular, the additives described in IT-A-20159 A/86, which have exhibited antirust properties, have the following structures: wherein R_{f} = ―CF₂R_{f}′CF₂―, R_{f}′ being a perfluoropolyether chain having an average molecular weight of 2000 and belonging to class (I).

The additives of the above types 1 and 3, however, exhibit the drawback of being scarcely soluble in the lubricating perfluoropolyether which causes problems with respect to phase separation, while the additive of type 2, although showing an acceptable solubility at the beginning, results in a certain amount of formed ester compounds in the course of time, whereby the mixture becomes cloudy and tends to form an overfloating layer. i.e., the additive separates from the lubricant.

There is, thus, a need to have available compounds capable of imparting to the lubricants to which they are added not only excellent antirust properties but also a long "shelf-life" (solubility of the additive retained in the course of time), which is absolutely necessary for the marketing of a lubricant.

It has, surprisingly, been found that the above properties may be achieved if, as an additive, a perfluoropolyether having a sequence of one or more of the following units is used:
wherein the groups R′_{f}, which may be the same or different from each other, are H or fluoroalkyl radicals (preferably having 1 to 3 carbon atoms such as, for example, CF₃ and C₂F₅) and having at least one end group selected from:

- (a): ―CFX-CN;
- (b): ―CFX-CH₂-NR₁R₂, wherein R₁ and R₂, the same or different from each other, represent H, C₁₋₈-, preferably C₁₋₄-alkyl, C₇₋₁₁-, preferably C₇₋₉-alkylaryl and C₆₋₁₀-, preferably C₆₋₈-cycloalkyl, optionally substituted with one or more C₁₋₃-alkyl groups; R₁ and R₂ optionally containing one or more heteroatoms selected from O, N and S;

wherein A = O, N or S and R is H or a C₁₋₃-alkyl group, particularly CH₃ and C₂H₅;
the group X in (a), (b) and (c) being F or CF₃;

The other end group may be one of the above groups (a), (b) and (c) but may also represent a perfluoroalkyl radical with 1 to 3 carbon atoms, for example, CF₃ or C₂F₅.

Some of these compounds are already described in US-A-4085137 for the preparation of polymers and as anti-corrosion agents. These compounds are not within the scope of the invention as claimed.

Examples of the various generic groups mentioned above are:

- C₁₋₈-alkyl:: Methyl, ethyl, n- and i-propyl, n-, i-, sek- and tert-butyl, pentyl, hexyl, heptyl and octyl; preferred are methyl and ethyl.
- C₇₋₁₁-alkylaryl:: Benzyl, phenylethyl, naphtylmethyl.
- C₆₋₁₀-cycloalkyl:: Cyclohexyl, cycloheptyl, cyclooctyl, cyclodecyl; preferred are cyclohexyl and cyclooctyl.
- C₁₋₃-alkyl;: see C₁₋₈-alkyl.

When A in group (c) is a nitrogen atom, the group attached thereto preferably has the same meanings as the groups R₁ and R₂, particularly H, CH₃ and C₂H₅.

In particular, preferred antirust additives of the present invention belong to the following classes:
wherein at least one of the end groups T and T′ is selected from:

- (a): ―CFX-CN;
- (b): ―CFX-CH₂-NR₁R₂, R₁ and R₂ being defined as above;
A and R being defined as above;
X in (a), (b) and (c) representing F or CF₃;
the other end group T or T′ may additionally be a perfluoroalkyl radical with 1 to 3 carbon atoms (for example, CF₃ or C₂F₅);
the indices g, h, m, n, k, j, p, q, s, t, r, u, v, z, x, y are integers selected in a manner such that the average molecular weight of the polyoxyfluoroalkylene chain ranges from 600 to 6000, preferably from 2000 to 4000 for difunctional compounds and from 1000 to 2000 for monofunctional compounds;
R_{f} is a fluoroalkylene radical preferably having 1 to 12, particularly 1 to 8 carbon atoms);
the groups R′_{f}, the same or different from each other, represent H or fluoroalkyl radicals (preferably having 1 to 3 carbon atoms);
the oxyfluoroalkylene units are statisticaly distributed along the chain.

Generally, the additives of the present invention exhibit a solubility in the PFPE lubricant of at least 1% by weight based on the lubricant.

The amount of the above fluoropolyether antirust additives preferably ranges from 1% to 5% by weight, based on the total lubricant amount, even more preferred from 2% to 4% by weight.

If the lubricant to which the antirust additive is added is a grease based on perfluoropolyethers, it may be prepared as is described in EP-A-92825.

In particular, such a grease can be formulated by suspending polytetrafluoroethylene particles having, for example, a spherical morphology and being composed of aggregates having a size of from 1 to 200 µm, in a liquid perfluoropolyether such as Fomblin ^{(R)}Y or Fomblin^{(R)}Z.

Due to their intrinsic lubricating properties the compounds having end groups of types (b) and (c) indicated above can also be utilized as such.

Furthermore, it has been found that the additives having the above end groups (a), (b) and (c) can be used in combination with small amounts of fluoropolyether compounds having the same chain structure as the compounds of the present invention, for example structures (I) to (XI), but one or two end groups ―CFX-COOH, wherein X is F or CF₃. Generally, the latter compounds are employed in amounts ranging from 1/30 to 1/20 (about 3 to about 5%) of the weight of the additive characterized by end groups (a), (b) and/or (c).

### The fluoropolyether precursors of the additives of the present invention may be prepared as follows:

- Class (I):: According to the processes described in US-A-3242218;
- Class (II):: According to US-A-3665041;
- Classes (III) and (IV):: According to EP-A-148482;
- Class (V):: According to US-A-4523039;
- Class (VI):: According to EP-A-151877;
- Class (VII):: According to US-A-3665041;
- Class (VIII):: According to US-A-3250808;
- Class (IX):: According to EP-A-148482;
- Class (X):: According to the processes described in PCT application WO87/00538;
- Class (XI):: According to the processes described in PCT application WO87/02992.

The above end groups can be introduced, for example, by the method described in US-A-3010874. In particular, the introduction of the end groups of type (a) may be effected by treating the corresponding derivatives with ester end groups ―CFX-COOR₃ (R₃ = CH₃, C₂H₅, C₆H₅) with anhydrous ammonia, preferably in a solvent such as, for example, ethyl ether, methanol or 1,1,2-trichlorotrifluoroethane, and subsequent treatment of the resulting amide with P₂O₅.

The introduction of end groups of types (b) and (c) may be effected by reacting the ester compounds indicated above with an amine of the formulae NHR₁R₂ or to form the corresponding amides and by subsequent reduction of the latter with hydrides.

In the case of classes (II), (III), (V), (VII), (VIII), (IX) and (X), in which the starting perfluoropolyethers have only one functional end group, it is possible to obtain the corresponding bifunctionalized product by means of the process described in EP-A-224201.

The antirust properties of the lubricants according to the present invention have been evaluated by means of the following tests:

### Antirust test in the fog chamber (method ASTM D.1748, modified)

### Object

Determination of the antirust properties of oils on metals in high humidity conditions.

### Summary of the method

Carbon steel plates (C15) (UNI), superficially treated as described below, were dipped into the oil, allowed to drip and hung in a fog chamber at 50°C and 100% relative humidity for a predetermined number of hours. The oil passes or does not pass the test on the basis of the number of rust stains visible on the surface of the plates.

### Apparatus

The fog chamber consisted of a compressed-air-actuated sprayer (P = 3 atm.), connected with a water reservoir so as to saturate the environment with humidity; the temperature was adjusted to 50°C (see ASTM B.117, 287, 368).

### Test conditions

The tests described below were carried out using partially demineralized water (pH = 5.5 to 7.5) and for the following periods of time:

- (1): The plates were hung and allowed to drip for 16 hours;
- (2): They were then placed into a fog chamber which was kept in operation for 8 hours;
- (3): The fog chamber was kept out of operation for 12 hours;
- (4): The fog chamber was turned on again and kept in operation for 8 hours;

Subsequently, the evaluation was made.

### Preparation of the steel plates

The steel plates were cleaned and degreased by means of a cloth soaked with Delifrene^{(R)} 113 (trichlorotrifluoroethane); the surface was polished by means of emery paper (400 mesh and 600˝), washed with water and dried. The utilized plates had the following dimensions: 50 × 100 × 2 mm. (Note: polyethylene gloves must be used to handle the plates).

### Evaluation of the tests (in analogy to method DIN 51802 (EMCOR) for bearings)

The results of the tests were expressed according to the following rating system:

- (0): No traces of rust were observed;
- (1): Very few corrosion points having a diameter below 1 mm;
- (2): 30% of the surface were covered by small stains having a diameter below 2 mm;
- (3): 60% of the surface were covered by small stains having a diameter below 3 mm;
- (4): 100% of the surface were covered by large stains having a diameter of 4 to 5 mm but the polished surface is visible in some points;
- (5): 100% of the surface were covered by large stains; the underlying surface is not visible.

In the evaluation, the rust stains appearing in the area up to 0.5 mm from the edges were not taken into consideration. With a rating of (0), the test was passed.

In the evaluation, two figures are given: The first figure refers to the state of the exposed face; The second figure refers to the non-exposed face (with respect to the sprayer).

The following examples merely serve to illustrate the invention and do not limit it in any way.

### EXAMPLE 1

Lubricants consisting of perfluoropolyethers having perfluoroalkyl end groups (Fomblin^{(R)}Y25), characterized by a viscosity of 250 cSt (250 mm²/s) at 20°C, to which the compounds indicated in the following Table 1 had been added, were subjected to the accelerated corrosion test in a fog chamber according to the method described above.

Table 1 shows the weight percentage of the additive with respect to the perfluoropolyether and the results of the corrosion test, expressed by the ratings (figures) outlined above.

### EXAMPLE 1A

Example 1 was repeated, using as lubricant perfluoropolyether Fomblin^{(R)}Y25 without additive. The result was a complete corrosion of the plate: 5-5.

### EXAMPLE 1B

Example 1 was repeated, using as lubricant Fomblin^{(R)}Y25 to which the following mixture had been added:
CH₂=CH-CH₂OCH₂CF₂O(CF₂CF₂O)ₘ(CF₂O)ₙCF₂CH₂OCH₂CH=CH₂
M.W. = 2000; 2%
HOOC-CF₂O(CF₂CF₂O)ₘ(CF₂O)ₙ-CF₂COOH
M.W. = 2000; 0.1%

This mixture was soluble in the perfluoropolyether but the result of the test was 3-2.

### EXAMPLE 2

Lubricants consisting of perfluoropolyethers having perfluoroalkyl end groups (Fomblin^{(R)}Z25), characterized by a viscosity of 250 cSt (250 mm²/s) at 20°C to which the compounds reported in the following Table 2 had been added were subjected to the accelerated corrosion test of example 1.

### Table 2 shows the results of said tests.

### EXAMPLE 2A

Example 2 was repeated, using as lubricant perfluoropolyether Fomblin^{(R)}Z25 without additive. The result was a complete corrosion of the plate: 5-5.

### EXAMPLE 2B

Example 2 was repeated, using as lubricant Fomblin^{(R)}Z25, to which the following mixture had been added:
CH₂=CH-CH₂OCH₂CF₂O(CF₂CF₂O)ₘ(CF₂O)ₙCF₂CH₂OCH₂CH=CH₂
M.W. 2000; 2%
HOOC-CF₂O(CF₂CF₂O)ₘ(CF₂O)ₙ-CF₂COOH
M.W. 2000; 0.1%

The test revealed a rather good anticorrosive effect (2-0) but the additive was insoluble in this type of perfluoropolyether.

### EXAMPLE 3

Subjected to the accelerated corrosion test of example 1 were the lubricants consisting of perfluoropolyethers having perfluoroalkyl end groups (Fomblin^{(R)}YR 140/13), characterized by a viscosity of 1400 cSt (1400 mm²/s) at 20°C to which the following mixture had been added:

The result of the corrosion test was 0-0.

### EXAMPLE 3A

Example 3 was repeated, using as lubricant perfluoropolyether Fomblin^{(R)}YR 140/13 without additive. The result was a complete corrosion of the plate: 5-5.

### EXAMPLE 3B

Example 3 was repeated, using as lubricant Fomblin^{(R)}YR 140/13, to which the following mixture had been added:
CH₂=CH-CH₂OCH₂CF₂O(CF₂CF₂O)ₘ(CF₂O)ₙCF₂CH₂OCH₂CH₂=CH₂
M.W. = 2000; 2%
HOOC-CF₂O(CF₂CF₂O)ₘ(CF₂O)ₙ-CF₂COOH
M.W. = 2000; 0.1%

The test revealed a rather good anticorrosive effect (1-0) but the additive was insoluble in this type of perfluoropolyether.

## Claims

1. Antirust additives for lubricants based on perfluoropolyethers, comprising one or more fluoropolyether compounds having one or more of the following units: wherein R′_{f} is H or a fluoroalkyl radical,
and having at least one end group selected from:
(a) ―CFX-CN;
(b) ―CFX-CH₂-NR₁R₂, wherein R₁ and R₂, the same or different from each other, are C₁₋₈-alkyl, C₇₋₁₁-alkylaryl or C₆₋₁₀-cycloalkyl groups, optionally substituted by C₁₋₃-alkyl groups, R₁ and R₂ optionally containing heteroatoms selected from O, N and S;
wherein A = O, N or S and R is H or a C₁₋₃-alkyl group;
the radical X in (a), (b) and (c) representing F or CF₃;
whereas the other end group has the meanings given above for the first end group or is a perfluoroalkyl radical having 1 to 3 carbon atoms; provided that in the case of fluoropolyether compounds having only units (Cf₂Cf₂O) and (Cf₂O) and one end group (a) or (b) the other end group is a perfluoroalkyl radical having 1 to 3 carbon atoms.

2. Additives according to claim 1, comprising one or more of the following fluoropolyether compounds: wherein at least one of the end groups T and T′ is selected from:
(a) ―CFX-CN;
(b) ―CFX-CH₂-NR₁R₂;
wherein X, R₁, R₂, A and R, are defined as in claim 1;
the other end group T or T′ can also be a perfluoroalkyl radical having 1 to 3 carbon atoms, and in the case of compound (I) has to be a perfluoroalkyl radical having 1 to 3 carbon atoms;
g, h, m, n, k, J, p, q, s, t, r, u, v, z, x, y are integers selected in a manner such that the average molecular weight of the polyoxyfluoroalkylene chain ranges from 600 to 6000; R_{f} is a fluoroalkylene radical; R′_{f} is H or a fluoroalkyl radical;
the oxyfluoroalkylene units are statistically distributed along the chain;
said additives having a solubility in the PFPE lubricant of at least 1% by weight based on the lubricant.

3. Additives according to claim 2, having a formula of type (I), end group of type (a) and an average molecular weight of about 2000.

4. Additives according to claim 2, having a formula of type (VII), end groups of type (c) and an average molecular weight of about 1000.

5. The use of fluoropolyether compounds having one or more of the following units as antirust additives for lubricants based on perfluoropolyethers; wherein R′_{f} is H or a fluoroalkyl radical,
and having at least one end group selected from:
(a) ―CFX-CN;
(b) ―CFX-CH₂-NR₁ R₂, wherein R₁ and R₂, the same or different from each other, are C₁₋₈-alkyl, C₇₋₁₁-alkylaryl or C₆₋₁₀-cycloalkyl groups, optionally substituted by C₁₋₃-alkyl groups, R₁ and R₂ optionally containing heteroatoms selected from O, N and S;
wherein A = O, N or S and R is H or a C₁₋₃-alkyl group;
the radical X in (a), (b) and (c) representing F or CF₃;
whereas the other end group has the meanings given above for the first end group or is a perfluoroalkyl radical having 1 to 3 carbon atoms.

6. The use according to claim 5, wherein one or more of the following fluoropolyether compounds are employed: wherein at least one of the end groups T and T′ is selected from:
(a) ―CFX-CN;
(b) ―CFX-CH₂-NR₁R₂;
wherein X, R₁, R₂, A and R, are defined as in claim 1;
the other end group T or T′ can also be a perfluoroalkyl radical having 1 to 3 carbon atoms;
g, h, m, n, k, j, p, q, s, t, r, u, v, z, x, y are integers selected in a manner such that the average molecular weight of the polyoxyfluoroalkylene chain ranges from 600 to 6000; R_{f} is a fluoroalkylene radical; R′_{f} is H or a fluoroalkyl radical;
the oxyfluoroalkylene units are statistically distributed along the chain;
said additives having a solubility in the PFPE lubricant of at least 1% by weight based on the lubricant.

7. The use according to claim 6, wherein fluoropolyether compounds having a formula of type (I), end groups of type (a) and an average molecular weight of about 2000 are employed.

8. Lubricants based on perfluoropolyethers having antirust properties, which contain the additives as defined in any one of claims 1 to 7.

9. Lubricants according to claim 8, wherein the additives are present in an amount ranging from 1 to 5% by weight, particularly from 2 to 4% by weight, based on the total amount of lubricant.

10. Lubricants according to any one of claims 8 and 9, additionally comprising fluoropolyether compounds having the same chain structure as the additives of claims 1 to 7, except that they show one or two end groups of the formula ―CFX-COOH, wherein X is F or CF₃, said additional additives being present in an amount ranging from 1/30 to 1/20 of the weight of the additives of claims 1 to 7.

## Patentansprüche

1. Rostschutzadditive für Schmiermittel auf Perfluorpolyetherbasis, umfassend eine oder mehrere Fluorpolyetherverbindungen, die eine oder mehrere der folgenden Einheiten aufweisen: worin R′_{f} H oder einen Fluoralkylrest darstellt,
und mindestens eine Endgruppe aufweisen, die ausgewählt ist aus:
(a) ―CFX-CN;
(b) ―CFX-CH₂-NR₁R₂, worin R₁ und R₂, gleich oder verschieden, C₁₋₈-Alkyl, C₇₋₁₁-Alkylaryl oder C₆₋₁₀-Cycloalkylgruppen, gegebenenfalls mit C₁₋₃-Alkylgruppen substituiert, darstellen, wobei R₁ und R₂ gegebenenfalls Heteroatome enthalten, die aus O, N und S ausgewählt sind;
worin A = O, N oder S und R H oder eine C₁₋₃-Alkylgruppe bedeutet;
wobei der Rest X in (a), (b) und (c) F oder CF₃ representiert;
während die andere Endgruppe die oben für die erste Endgruppe angegebene Bedeutung hat oder einen Perfluoralkylrest mit 1 bis 3 Kohlenstoffatomen darstellt;
mit der Maßgabe, daß im Fall von Fluorpolyetherverbindungen, die lediglich die Einheiten (CF₂CF₂O) und (CF₂O) und eine Endgruppe (a) oder (b) aufweisen, die andere Endgruppe einen Perfluoralkylrest mit 1 bis 3 Kohlenstoffatomen darstellt.

2. Additive nach Anspruch 1, umfassend eine oder mehrere der folgenden Fluorpolyetherverbindungen: worin mindestens eine der Endgruppen T und T′ ausgewählt ist aus:
(a) ―CFX-CN;
(b) ―CFX-CH₂-NR₁R₂;
worin X, R₁, R₂, A und R wie in Anspruch 1 definiert sind;
die andere Endgruppe T oder T′ ebenfalls ein Perfluoralkylrest mit 1 bis 3 Kohlenstoffatomen sein kann, und im Fall der Verbindung (I) ein Perfluoralkylrest mit 1 bis 3 Kohlenstoffatomen sein muß;
g, h, m, n, k, j, p, q, s, t, r, u, v, z, x, y ganze Zahlen sind, derart ausgewählt, daß das durchschnittliche Molekulargewicht der Polyoxyfluoralkylenkette 600 bis 6000 beträgt; R_{f} ein Fluoralkylenrest ist; R′_{f} H oder einen Fluoralkylrest bedeutet;
die Oxyfluoralkyleneinheiten statistisch entlang der Kette verteilt sind;
wobei die Additive eine Löslichkeit im PFPE-Schmiermittel von mindestens 1 Gew.-%, bezogen auf das Schmiermittel, aufweisen.

3. Additive nach Anspruch 2 mit einer Formel vom Typ (I), einer Endgruppe vom Typ (a) und einem durchschnittlichen Molekulargewicht von etwa 2000.

4. Additive nach Anspruch 2 mit einer Formel vom Typ (VII), Endgruppen vom Typ (c) und einem durchschnittlichen Molekulargewicht von etwa 1000.

5. Verwendung von Fluorpolyetherverbindungen als Rostschutzadditive für Schmiermittel auf Perfluorpolyetherbasis, die eine oder mehrere der folgenden Einheiten aufweisen: worin R′_{f} H oder einen Fluoralkylrest darstellt,
und mindestens eine Endgruppe aufweisen, die ausgewählt ist aus:
(a) ―CFX-CN;
(b) ―CFX-CH₂-NR₁R₂, worin R₁ und R₂, gleich oder verschieden, C₁₋₈-Alkyl, C₇₋₁₁-Alkylaryl oder C₆₋₁₀-Cycloalkylgruppen, gegebenenfalls mit C₁₋₃-Alkylgruppen substituiert, darstellen, wobei R₁ und R₂ gegebenenfalls Heteroatome enthalten, die aus O, N und S ausgewählt sind;
worin A = O, N oder S und R H oder eine C₁₋₃-Alkylgruppe bedeutet;
wobei der Rest X in (a), (b) und (c) F oder CF₃ repräsentiert;
während die andere Endgruppe die oben für die erste Endgruppe angegebene Bedeutung hat oder einen Perfluoralkylrest mit 1 bis 3 Kohlenstoffatomen darstellt.

6. Verwendung nach Anspruch 5, worin eine oder mehrere der folgenden Fluorpolyetherverbindungen eingesetzt werden: worin mindestens eine der Endgruppen T und T′ ausgewählt ist aus:
(a) ―CFX-CN;
(b) ―CFX-CH₂-NR₁R₂;
worin X, R₁, R₂, A und R wie in Anspruch 1 definiert sind;
die andere Endgruppe T oder T′ ebenfalls ein Perfluoralkylrest mit 1 bis 3 Kohlenstoffatomen sein kann;
g, h, m, n, k, j, p, q, s, t, r, u, v, z, x, y ganze Zahlen sind, derart ausgewählt, daß das durchschnittliche Molekulargewicht der Polyoxyfluoralkylenkette 600 bis 6000 beträgt; R_{f} ein Fluoralkylenrest ist; R′_{f} H oder einen Fluoralkylrest bedeutet;
die Oxyfluoralkyleneinheiten statistisch entlang der Kette verteilt sind;
wobei die Additive eine Löslichkeit im PFPE-Schmiermittel von mindestens 1 Gew.-%, bezogen auf das Schmiermittel, aufweisen.

7. Verwendung nach Anspruch 6, worin Fluorpolyetherverbindungen mit einer Formel vom Typ (I), Endgruppen vom Typ (a) und einem durchschnittlichen Molekulargewicht von etwa 2000 eingesetzt werden.

8. Schmiermittel auf Perfluorpolyetherbasis mit Rostschutzeigenschaften, welche die Additive nach irgendeinem der Ansprüche 1 bis 7 enthalten.

9. Schmiermittel nach Anspruch 8, worin die Additive in einer Menge von 1 bis 5 Gew.-%, vorzugsweise 2 bis 4 Gew.-%, bezogen auf die Gesamtmenge des Schmiermittels, anwesend sind.

10. Schmiermittel nach irgendeinem der Ansprüche 8 und 9, die zusätzlich Fluorpolyetherverbindungen umfassen, welche dieselbe Kettenstruktur wie die Additive der Ansprüche 1 bis 7 aufweisen, mit der Ausnahme, daß sie 1 oder 2 Endgruppen der Formel ―CFX-COOH haben, worin X F oder CF₃ ist, wobei die zusätzlichen Additive in einer Menge von 1/30 bis 1/20 des Gewichts der Additive nach Anspruch 1 bis 7 vorhanden sind.

## Revendications

1. Additifs antirouille pour lubrifiants à base de perfluoropolyéthers comprenant un ou plusieurs composés fluoropolyéthers ayant un ou plusieurs des motifs suivants: où les groupes R′_{f} représentent chacun H, ou un radical fluoroalkyle et comporte au moins un groupe terminal choisi parmi:
(a) ―CFX-CN;
(b) ―CFX-CH₂-NR₁R₂, où R₁ et R₂, identiques ou différents, représentent chacun un groupe H, alkyle en C₁₋₈, alkyl-aryle en C₇₋₁₁ ou cycloalkyle en C₆₋₁₀, éventuellement substitué par un ou plusieurs groupes alkyles en C₁₋₃; R₁ et R₂ pouvant facultativement contenir un ou plusieurs hétéroatomes choisis parmi O, N et S;
où:
A = O, N ou S; et
R est H ou un groupe alkyle en C₁₋₃;
le radical X, dans (a), (b) et (c) étant F ou CF₃,
l'autre groupe terminal ayant les significations données ci-dessus pour le premier groupe terminal ou étant un radical perfluoralkyle ayant 1 à 3 atomes de carbone; à la condition que, quand les composés fluoropolyéthers ne comportent que des motifs (CF₂CF₂O) et (CF₂O) et un groupe terminal (a) ou (b), l'autre groupe terminal soit un radical perfluoralkyle ayant de 1 à 3 atomes de carbone.

2. Additifs selon la revendication 1 comprenant un ou plusieurs des composés fluoropolyéthers suivants: où au moins l'un des groupes terminaux T et T′ est choisi parmi:
(a) ―CFX-CN;
(b) ―CFX-CH₂-NR₁R₂, R₁ et R₂ sont tels que définis ci-dessus;
où X, R₁, R₂, A et R sont tels que définis dans la revendication 1;
l'autre groupe terminal T ou T′ pouvant aussi être un radical perfluoralkyle ayant 1 à 3 atomes de carbone et, dans le cas du composé (I), devant être un radical perfluoroalkyle ayant 1 à 3 atomes de carbone;
g, h, m, n, k, j, p, q, s, t, r, u, v, z, x et y étant des nombres entiers choisis de façon que la masse moléculaire moyenne de la chaîne polyoxyfluoralkylène soit comprise entre 600 et 6000;
R_{f} étant un radical fluoralkylène;
R′_{f} étant H ou un radical fluoralkyle;
les motifs fluoralkylènes étant statistiquement distribués le long de la chaîne;
lesdits additifs ayant dans le lubrifiant au PFPE une solubilité d'au moins 1% en poids par rapport au lubrifiant.

3. Additifs selon la revendication 2, ayant une formule de type (I), un groupe terminal de type (a) et une masse moléculaire moyenne d'environ 2000.

4. Additifs selon la revendication 2, ayant une formule de type (VII), des groupes terminaux de type (c) et une masse moléculaire moyenne d'environ 1000.

5. L'utilisation de composés fluoropolyéthers ayant un ou plusieurs des motifs suivants, en tant qu'additifs antirouille pour lubrifiants à base de perfluoropolyéthers: où les groupes R′_{f} représentent chacun H, ou un radical fluoroalkyle et comporte au moins un groupe terminal choisi parmi:
(a) ―CFX-CN;
(b) ―CFX-CH₂-NR₁R₂, où R₁ et R₂, identiques ou différents, représentent chacun un groupe H, alkyle en C₁₋₈, alkyl-aryle en C₇₋₁₁ ou cycloalkyle en C₆₋₁₀, éventuellement substitué par un ou plusieurs groupes alkyles en C₁₋₃; R₁ et R₂ pouvant facultativement contenir un ou plusieurs hétéroatomes choisis parmi O, N et S;
où
A = O, N ou S; et
R est H ou un groupe alkyle en C₁₋₃;
le radical X, dans (a), (b) et (c) étant F ou CF₃, l'autre groupe terminal ayant les significations données ci-dessus pour le premier groupe terminal ou étant un radical perfluoralkyle comportant 1 à 3 atomes de carbone.

6. L'utilisation selon la revendication 5, dans laquelle on utilise un ou plusieurs des composés perfluoropolyéthers suivants: où au moins l'un des groupes terminaux T et T′ est choisi parmi:
(a) ―CFX-CN;
(b) ―CFX-CH₂-NR₁R₂, R₁ et R₂ sont tels que définis ci-dessus;
où X, R₁, R₂, A et R sont tels que définis dans la revendication 1;
l'autre groupe terminal T ou T′ pouvant aussi être un radical perfluoralkyle ayant 1 à 3 atomes de carbone;
g, h, m, n, k, j, p, q, s, t, r, u, v, z, x et y étant des nombres entiers choisis de façon que la masse moléculaire moyenne de la chaîne polyoxyfluoralkylène soit comprise entre 600 et 6000;
R_{f} étant un radical fluoralkylène;
R′_{f} étant H ou un radical fluoralkyle;
les motifs fluoralkylènes étant statistiquement distribués le long de la chaîne;
lesdits additifs ayant dans le lubrifiant au PFPE une solubilité d'au moins 1% en poids par rapport au lubrifiant.

7. L'utilisation selon la revendication 6, dans laquelle on utilise des composés fluoropolyéthers ayant une formule de type (I), des groupes terminaux de type (a) et une masse moléculaire moyenne d'environ 2000.

8. Lubrifiants à base de perfluoropolyéthers, ayant des propriétés antirouille, qui contiennent les additifs tels que définis dans l'une quelconque des revendications 1 à 7.

9. Lubrifiants selon la revendication 8, dans lesquels les additifs sont présents en une quantité de 1 à 5% en poids, en particulier de 2 à 4% en poids par rapport à la quantité totale de lubrifiant.

10. Lubrifiants selon l'une quelconque des revendications 8 et 9, comprenant en outre des composés fluoropolyéthers ayant la même structure de chaîne que les additifs des revendications 1 à 7, sauf qu'ils comportent un ou deux groupes terminaux de formule ―CFX-COOH, dans laquelle X est F ou CF₃, lesdits additifs supplémentaires étant présents en une quantité comprise entre 1/30è et 1/20è du poids des additifs des revendications 1 à 7.
